

Oct. 7, 1958

L. W. RAINARD

2,854,701

## CRIMPING METHOD AND APPARATUS

Filed March 7, 1956



1

2,854,701

## CRIMPING METHOD AND APPARATUS

Leo W. Rainard, Wilmington, Del., assignor to Joseph Bancroft & Sons Co., Wilmington, Del., a corporation of Delaware

Application March 7, 1956, Serial No. 570,145

8 Claims. (Cl. 19—66)

This invention relates to a method and apparatus for producing a permanent artificial crimp in textile fibers.

The invention is applicable to cellulosic textile fibers and provides a novel and improved means for producing in such fibers a permanent crimp of the saw tooth type in which the fibers are formed into a series of angular bends separated by straight fiber lengths or legs. Such a crimp may be produced in a stuffer crimper wherein the fibers to be crimped are fed between feed rolls into a closed crimping chamber against a mass of crimped fibers held compacted in said chamber so that the fibers are folded over into a zig-zag crimp as they leave the bite of the feed rolls. The crimped fibers are continuously advanced to the discharge end of said chamber at a predetermined rate dependent upon the length of time the fibers are to remain in the chamber and during which time the setting operation of the present invention takes place.

The fibers or yarns may be in the form of a rope or sliver composed of carded staple fibers or may be in the form of a bundle of continuous filaments which may or may not be twisted into yarn. The invention is applicable for example to regenerated cellulose rayon, cotton, linen, hamp, ramie, jute, and the like.

In accordance with this invention the fibers are impregnated with an impregnant capable of fixing the crimped effect upon heating the impregnated fiber. Such impregnant may be any one of a wide variety of materials, either a thermosetting resin precondensate such as dimethylol melamine or an impregnant adapted to react with the fiber itself upon heating in the curing zone, such as dimethylol ethylene urea. Usually, such impregnation is effected by application of an aqueous solution of the resin materials, followed by drying the fibers to provide a moist condition.

The nature of the impregnant employed may be varied without departing from the scope of the invention, the important consideration being that the impregnant be capable of fixing the crimp upon heating the impregnated crimped fibers so that the set is not affected by subsequent washing or steaming or by other conditions normally encountered in the use or fabrication of the fibers.

The fibers are impregnated while in the crimping chamber or prior to being fed to the crimping chamber and the impregnant is cured while the fibers are held compacted in the crimping chamber, at least to a point such that the crimp is retained when the compacting force is released. The complete curing may be effected in the crimping chamber or in a separate curing zone.

The invention will be better understood by referring to the following description, taken in connection with the accompanying drawing in which a specific embodiment has been set forth for purposes of illustration.

In the drawing:

Fig. 1 is a diagrammatic view of an apparatus embodying the invention with parts shown in section; and

2

Fig. 2 is a section on a larger scale taken on the line 2—2 of Fig. 1.

Referring to the drawing more in detail the filament tow or yarn 10 is passed through feed rolls 11 into an impregnation solution 12 in a tank 13. The impregnated yarn is removed from the solution 12 through squeeze rolls 14 which remove the excess solution and is fed through a drier 15 and around guide rolls 16 to a guide 17 which directs the impregnated and dried yarn into the stuffer crimper.

The stuffer crimper is shown as comprising heater blocks 20, 21 and 22 mounted on a supporting plate 24 and formed with cylindrical bores in which sleeves 25, 26 and 27 respectively are secured.

The plate 24 carries a bearing in which is journaled a shaft 28 carrying a feed roll 29. A second feed roll 30 is carried by a shaft 31 journaled in a bearing in an arm 32 which is pivotally attached by a pin 33 to a bracket 34 which is attached to or carried by the plate 24. The shaft 28 is driven by a source of power such as a motor not shown. The shaft 31 is driven in unison therewith by meshing gears 35 and 36 carried by the respective shafts 28 and 31.

The feed rolls 29 and 30 are held in pressure engagement with the yarn 10 by means of a spring 37 attached at one end to a post 38 on the arm 32 and at the other end to a post 39 on the plate 24. Adjustment is provided by a threaded pin 40 and nut 41.

The yarn 10 is guided to the bite of the feed rolls 29 and 30 by the guide 17 which is attached by a screw 42 to the plate 24. The lower end of sleeve 25 is slotted to receive the rolls 29 and 30 and extends below the bite of the rolls to form therewith a substantially closed crimping chamber into which the yarn 10 is fed for crimping.

The blocks 20, 21 and 22 may be heated by suitable means such as by Calrod units 45, 46 and 47 respectively which are inserted in bores in blocks 20, 21 and 22 and extend parallel to the sleeves 25, 26 and 27 so as to heat the walls of the sleeves. The Calrods may be controlled so as to heat the yarn in the sleeves to the temperature necessary for curing the impregnant above described.

The sleeves 25, 26 and 27 are joined by collars 50 and 51 which may be threaded for ease of assembly. The collars 50 and 51 are formed with ports 52 and 53 communicating with pipes 54 and 55 respectively through which fluid can be introduced. The rate of flow of such fluid can be regulated by metering valves 56 and 57 respectively.

The sleeve 25 below the heater block 20 is provided with a plurality of inlet ports 60 which are disposed radially around the periphery thereof and communicate with an eccentric annular groove 61 in the outer periphery of the sleeve 25. A coupling ring 62 is clamped around the sleeve 25 in alignment with the annular groove 61 by a clamping screw 63 and carries a pipe 64 having a metering valve 65 by which a fluid may be introduced through the ports 60 into the interior of the sleeve 25.

A plug 68 is inserted in the top of the sleeve 27 to rest upon the crimped yarn 69 within the sleeve. The plug 68 may be provided with a bore 70 through which the crimped yarn 69 is withdrawn by take-up rolls 71 which may be operated at a constant rate bearing a predetermined relationship to the rate of feed of the yarn 10 by the feed rolls 29 and 30, which relationship may be adjusted in response to variations in the portion of the plug 68, so as to maintain the plug at a constant level within the sleeve 27.

From the take-up rolls 71 the crimped yarn 69 may be fed to an oven 73 which is maintained at a temperature adapted for the final curing of the impregnant. The

crimp set yarn may be removed from the oven 73 by take-up rolls 74 and fed to a winding device not shown.

To permit the escape of steam or vapor during the heating of the fibers the sleeves 25, 26 and 27 are provided within the blocks 20, 21 and 22 with a plurality of sets of radial exhaust ports 76, 77 and 78 respectively which are disposed around the periphery of the sleeves and register with exhaust passages 79, 80 and 81 respectively in the blocks 20, 21 and 22.

In the operation of this process the tow or yarn 10 to be crimped is first treated with the impregnant solution 12 in the tank 13 and is dried to a moist state by the drier 15. The impregnated and dried tow or yarn is then fed by feed rolls 29 and 30 into the crimping chamber formed by the sleeve 25 against the pressure exerted by the mass of crimped yarn in the chamber. A suitable catalyst may be introduced into the mass of fibers through the pipe 64 or the pipe 54 or through both pipes as required.

If the catalyst is introduced through the lower pipe 64 the fibers are cured in the sleeves 25, 26 and 27. If the catalyst is introduced through the pipe 54 the fibers dried in the sleeve 25 are cured in the sleeves 26 and 27.

As the fibers advance through the sleeves 25, 26 and 27 they are heated to a predetermined temperature suited for curing or partially curing the impregnant. The time that the fibers are exposed to the curing temperature is dependent upon the rate of feed by the feed rolls 29 and 30 and upon the length of the heated portion of the sleeves.

The pretreatment in the tank 13 and drier 15 may be omitted if sufficient dwell is provided in the crimper itself in which case the fibers are fed directly to the feed rolls 29 and 30, the impregnant is introduced through the pipe 64, dried in the sleeve 25, the catalyst introduced through pipes 54 and the impregnant cured in the sleeves 26 and 27. If further drying is required between the impregnation and the introduction of the catalyst the impregnant may be introduced through the pipe 64, the fibers dried in the sleeves 25 and 26, the catalyst introduced through the pipe 55 and cured in the sleeve 27.

In a further embodiment the impregnant and catalyst may be introduced together, either in the tank 13 or through the pipe 64. The order of introduction may also be reversed, the catalyst being introduced first and the impregnant at a later stage followed by curing in the crimper.

It is possible to impregnate the fibers in tank 13 with one of the chemicals used in making the precondensate, for example urea, and then to introduce the others, for example formaldehyde, through pipe 64. The catalyst may be added to either ingredient or introduced separately through pipe 54 or 55.

If the curing is complete in the sleeves 25 and 26 the block 22 may be cooled instead of heated so as to cool the fibers to a temperature to stop the reaction before the yarn is wound onto a package.

In some cases a softening or lubricating agent may be introduced through the upper pipe 55 followed by drying in the sleeve 27.

The upper portion of the sleeve 27 which extends above the block 22 constitutes a cooling zone in which the fibers are cooled before being removed from the crimper. In the event that the curing is not complete in the sleeve 27 and further curing is to be effected in the oven 73, the intermediate cooling zone in the upper portion of the sleeve 27 may be eliminated by making the sleeve terminate as closely as possible at the top of the heated block 22. If final curing takes place in the oven 73 additional impregnant material may be introduced through the upper pipe 55.

Following are various examples of the sequence of steps which may be used in carrying out this invention:

(1) The yarns may be impregnated, squeezed, partially dried before entering the crimping chamber, then crimped and cured in the crimping chamber.

(2) The yarns may be impregnated and squeezed before entering the crimping chamber, then crimped, dried and cured in the crimping chamber.

(3) The yarns may be impregnated and partially dried before entering the crimping chamber, then crimped and the catalyst introduced through lower inlet pipe 64 or intermediate inlet pipe 54.

(4) The catalyst may be introduced in the tank 13 or through the lower pipe 64, directly in sleeve 25, the impregnant introduced through pipe 54 or 55 and cured in the crimping chamber.

(5) The yarns may be crimped and the impregnant be injected through pipe 64 or 54, dried and cured in the crimping chamber.

(6) The yarn may be crimped, the impregnant injected through pipe 55, partially cured in sleeve 27 and finally cured in oven 73.

(7) The yarn may be crimped and the impregnant injected through pipe 64, dried, the catalyst injected through pipe 54 or 55, dried and cured in the sleeve 27, or partially cured in sleeve 27, and finally cured in oven 73.

(8) The yarn may be crimped, the catalyst injected through pipe 64, dried, the impregnant injected through pipe 54 or 55, and dried and cured in the sleeve 27.

(9) In any of the above combinations a softening agent or a lubricant may be introduced through the pipe 54 or 55 or into the top of the sleeve 27.

Types of amino-plast resin impregnants which can be used are as follows: Urea formaldehyde types having formaldehyde urea mol ratios from 1:1 to 2:1, such as sesquimethylol urea; modified urea formaldehyde, such as dimethylol ethylene urea, dimethylol 1,2 propylene urea, dimethylol 1,2 butylene urea, dimethylol 3,4 butylene urea; methylol melamine resins, such as mixtures of dimethylol and trimethylol melamines or mixtures of tetramethylol and pentamethylol melamines; methylated-methylol melamines, such as dimethyl trimethylol melamines.

The following examples are based on 100% pickups of the fibers:

Example I:

20 lbs. dimethylol urea  
32 lbs. methylated methylol melamine  
20 lbs. cationic softener  
20 lbs. catalyst  
Add water to make 100 gallons.

Example II:

45 lbs. dimethylol urea  
20 lbs. cationic softener  
20 lbs. catalyst  
Add water to make 100 gallons.

Example III:

60 lbs. methylated methylol melamine  
20 lbs. cationic softener  
20 lbs. catalyst  
Add water to make 100 gallons.

Example IV:

40 lbs. methylated methylol melamine  
25 lbs. dimethylol urea  
15 lbs. cationic softener  
20 lbs. catalyst  
4 lbs. polyvinyl alcohol (99% hydrolyzed)  
Add water to make 100 gallons.

Example V:

15 lbs. methylated methylol melamine  
24 lbs. dimethylol urea  
20 lbs. cationic softener  
16 lbs. catalyst  
2 lbs. polyvinyl alcohol (99% hydrolyzed)  
Add water to make 100 gallons.

## Example VI:

40 lbs. methylated methylol melamine  
 20 lbs. cationic softener  
 18 lbs. catalyst  
 2 lbs. polyvinyl alcohol (99% hydrolyzed)  
 Add water to make 100 gallons.

## Example VII:

56 lbs. methylated methylol melamine  
 20 lbs. cationic softener  
 22 lbs. catalyst  
 2 lbs. polyvinyl alcohol (99% hydrolyzed)  
 Add water to make 100 gallons.

## Example VIII:

30 lbs. sesquimethylol urea  
 30 lbs. dimethylol ethylene urea  
 20 lbs. cationic softener  
 20 lbs. catalyst  
 Add water to make 100 gallons.

## Example IX:

60 lbs. methylated methylol melamine  
 20 lbs. cationic softener  
 20 lbs. catalyst  
 100 lbs. water

A suitable cationic softener is s-Di 1-(2 stearamidoethyl) urea mono acetate. However, other cationic softeners, such as dimethyl ammonium methyl sulfate or monostearylmetaphenylene diamine would be satisfactory.

The catalyst generally used is a 70% solution of magnesium chloride hexahydrate. However, several other catalysts, such as methylhydroxypropanolamine hydrochloride may be satisfactorily used. Certain types of catalysts could even be utilized in the gaseous state, such as hydrogen chloride which in the presence of water would be acidic. The invention is not to be limited as to catalyst since any of the catalysts commonly used with thermosetting resins may be used.

The composition of Example II is preferred for regenerated cellulose rayon. The remaining examples are satisfactory for the other cellulosics.

In processes in which the catalyst is to be introduced separately it would be removed from the formulation, and a more concentrated solution would be injected into the inlet orifices. For example, the formula of Example 1 may be separated into (a) an impregnant consisting of:

20 lbs. methylated methylol melamine  
 32 lbs. dimethylol urea  
 20 lbs. cationic softener  
 Add water to make 100 gallons.

and (b) 21 lbs. of catalyst dissolved in 21 lbs. of water which is separately injected at a rate to inject 5 grams of catalyst while 100 grams of yarn are passing the injection port in a given length of time.

The impregnant may be injected at a rate so that 100 grams would be injected during the time that 100 grams of yarn are passing the port. The concentration of the ingredients in the impregnant may be increased and the rate of injection decreased if so desired.

Cotton yarn or rayon may be impregnated with any of the above mixtures, squeezed to leave about a 100% increase in weight, partially dried to a 10% to 15% moisture content and crimped in a stuffer crimpler. The crimped fiber is maintained in the crimping chamber at a temperature above 290° F. for a period of about 2½ minutes. The time and temperature may be varied inversely. For example the fibers may be held in the crimping chamber for from five minutes to a half of a

minute at temperatures varying from 200° F. to 450° F. The shorter time being coupled with the higher temperatures and vice versa. Under the above conditions the resin is completely cured before the fibers leave the crimping chamber and produces a permanently set crimp which is resistant to washing and boiling.

What is claimed is:

1. The method of imparting a permanently set crimp to cellulosic textile fibers, which comprises feeding said fibers continuously in the form of a tow or yarn into a closed crimping zone against a mass of crimped fibers held compacted in said zone to cause the fibers to fold and form zig-zag crimps as they contact said mass of crimp fibers, advancing the crimped fibers along said zone to a discharge point, applying to the fibers at a point in advance of their discharge point a resinous impregnant capable of setting the crimp in said fibers under the action of heat, applying heat to said crimped fibers, as said crimped fibers pass through said zone, at a plurality of sequential heating areas and feeding a catalyst for said resinous material into said zone in advance of at least one of said heating areas, whereby permanent setting of the crimp in said fibers is effected prior to the removal of said crimp fibers from said discharge point.
2. The method set forth in claim 1 in which the fibers are treated with said impregnant before being fed into said crimping zone.
3. The method set forth in claim 1 in which the fibers are treated with said impregnant and at least partially dried before being fed into said crimping zone.
4. The method set forth in claim 1 in which the impregnant is introduced into said crimping zone.
5. The method set forth in claim 1 in which the crimped fibers are fed from said crimping zone into an oven for the final curing of said impregnant.
6. Crimping apparatus comprising a tube forming a crimping chamber, a pair of feed rolls disposed to feed fibers for crimping into one end of said tube, a closure member disposed to control the discharge of crimped fibers from the other end of said tube, heating means to heat said tube for a portion of its length to provide a heating zone for the fibers within said tube, said tube having an inlet port for a treating fluid in advance of said heating zone, an exhaust port in said heating zone, and a second inlet port disposed beyond said exhaust ports in said heating zone, and a third inlet port beyond said second inlet port in the direction of travel of said fibers in said tube.
7. Crimping apparatus comprising a tube forming a crimping chamber, a pair of feed rolls disposed to feed fibers for crimping into one end of said tube, a closure member disposed to control the discharge of crimped fibers from the other end of said tube, heating means to heat said tube for a portion of its length to provide a heating zone for the fibers within said tube, said tube having an inlet port for a treating fluid in advance of said heating zone, a plurality of exhaust ports disposed along said heating zone, and a second inlet port disposed beyond said exhaust ports in said heating zone.
8. Crimping apparatus comprising a tube forming a crimping chamber, a pair of feed rolls disposed to feed fibers for crimping into one end of said tube, a closure member disposed to control the discharge of crimped fibers from the other end of said tube, heating means to heat said tube for a portion of its length to provide a heating zone for the fibers within said tube, said tube having an inlet port for a treating fluid in advance of said heating zone, a plurality of exhaust ports disposed along said heating zone, and a second inlet port disposed beyond said exhaust ports in said heating zone, and a third inlet port beyond said second inlet port in the direction of travel of said fibers in said tube.

## References Cited in the file of this patent

## UNITED STATES PATENTS

2,363,019 Schurmann et al. Nov. 21, 1944  
2,556,011 Swayze et al. June 5, 1951

2,575,781 Barach Nov. 20, 1951  
2,623,266 Hemmi Dec. 30, 1952  
2,669,001 Keen Feb. 16, 1954  
2,733,122 Herele et al. Jan. 31, 1956  
2,734,228 Hay Feb. 14, 1956